

## UNITED STATES PATENT OFFICE

2,494,597

## VINYL AIR-DRYING WRINKLE COMPOSITION AND METHOD OF APPLYING SAME

William A. Waldie, Dayton, Ohio, assignor to New Wrinkle, Inc., Dayton, Ohio, a corporation of Delaware

No Drawing. Application February 28, 1947,  
Serial No. 731,718

5 Claims. (Cl. 117—41)

1

This invention deals with a wrinkle coating composition and a method of coating articles therewith.

It is an object of this invention to prepare coating compositions which yield a wrinkle-textured film from solutions of non-wrinking resins.

It is another object of this invention to prepare wrinkle coating compositions without the use of any heating or cooking steps.

It is still another object of this invention to prepare wrinkle coating compositions which yield a film of great homogeneity.

These and other objects are accomplished by mixing polyvinyl butyral, butanol and water. This type of mixture, when applied to a surface and dried, yields a texture of very uniform wrinkle formation.

While polyvinyl butyral dissolved in butanol yields an entirely smooth surface upon drying, the addition of water causes formation of wrinkles. This result was wholly unexpected and surprising.

In the following, one example is given of a composition according to my invention which yielded especially satisfactory results.

## Example

4 lbs. polyvinyl butyral  
4 gals. butanol  
1 gal. water

The mixture is prepared by blending the ingredients at room temperature. It is advisable to let the mixture stand for a short while until air bubbles which are usually occluded have escaped. Thereafter, the mixture is ready for application to the articles to be coated which may be done by any method customary in the art such as spraying, immersing, knifing and the like. The solvent is then removed from the coating by baking or air drying. Baking may be carried out by means of a gas heated or electrical oven or by infrared light. If infrared heat is applied, a heating time of from 1 to 5 minutes is usually sufficient. It is obvious that also a combination of various kinds of heating may be used; thus, for example, air drying for 45 minutes with subsequent oven drying at 200 to 212° F. for approximately ½ hour yielded also films of great uniformity and satisfactory hardness. However, air drying for approximately 3 hours is about the simplest and cheapest method, and the same satisfactory result, namely a film of sufficient hardness and uniformity of the wrinkles is obtained thereby.

It will be understood that conventional additional materials such as plasticizers, pigments, dyes or the like may be added to the new composi-

2

tion without departing from the scope of the invention.

It will also be understood that while there have been described herein certain specific embodiments of the invention, it is not intended thereby to have it limited to or circumscribed by the specific details given in view of the fact that this invention is susceptible to various modifications and changes which come within the spirit of this disclosure and the scope of the appended claims.

I claim:

1. A wrinkle coating composition consisting of a mixture of 4 lbs. of polyvinyl butyral, 4 gals. of butanol and 1 gal. of water.

2. In a method of coating articles with a wrinkle-textured film, the steps of preparing a mixture consisting of from 4 lbs. of polyvinyl butyral, 4 gals. of butanol and 1 gal. of water; allowing air to escape from said mixture; applying said mixture to the surface to be coated; and drying said coating whereby a wrinkle-textured film is obtained.

3. In a method of coating articles with a wrinkle-textured film, the steps of preparing a mixture consisting of from 4 lbs. of polyvinyl butyral, 4 gals. of butanol and 1 gal. of water; allowing air to escape from said mixture; applying said mixture to the surface to be coated; and drying said coating with infrared heat for from 1 to 5 minutes.

4. In a method of coating articles with a wrinkle-textured film, the steps of preparing a mixture consisting of from 4 lbs. of polyvinyl butyral, 4 gals. of butanol and 1 gal. of water; allowing air to escape from said mixture; applying said mixture to the surface to be coated; and drying said coating at room temperature for approximately 45 minutes and thereafter to 200—212° F. for about ½ hour.

5. In a method of coating articles with a wrinkle-textured film, the steps of preparing a mixture consisting of from 4 lbs. of polyvinyl butyral, 4 gals. of butanol and 1 gal. of water; allowing air to escape from said mixture; applying said mixture to the surface to be coated; and air drying said coating for approximately 3 hours.

WILLIAM A. WALDIE.

## REFERENCES CITED

The following references are of record in the file of this patent:

## UNITED STATES PATENTS

| Number    | Name            | Date          |
|-----------|-----------------|---------------|
| 1,746,665 | Matheson et al. | Feb. 11, 1930 |
| 1,971,951 | Skirrow et al.  | Aug. 28, 1934 |
| 2,321,939 | Quinn           | June 15, 1943 |